

# United States Patent

Barrett

[15] 3,671,409

[45] June 20, 1972

## [54] ELECTRODEPOSITION OF NICKEL

[72] Inventor: Ernest Charles Henry Barrett, Thornton Heath, England

[73] Assignee: London & Scandinavian Metallurgical Co., Limited, London, England

[22] Filed: May 4, 1970

[21] Appl. No.: 34,638

## [30] Foreign Application Priority Data

May 7, 1969 Great Britain ..... 23,285/69

[52] U.S. Cl. ..... 204/49

[51] Int. Cl. ..... C23b 5/08

[58] Field of Search ..... 204/49

## [56] References Cited

### UNITED STATES PATENTS

3,244,603 5/1966 Stephenson et al. ..... 204/43

3,271,274 9/1966 Giulio et al. ..... 204/43

3,454,376 7/1969 Luce et al. ..... 204/49

3,489,660 1/1970 Semienko et al. ..... 204/43

## FOREIGN PATENTS OR APPLICATIONS

|           |        |                    |        |
|-----------|--------|--------------------|--------|
| 902,499   | 8/1962 | Great Britain..... | 204/49 |
| 1,059,915 | 2/1967 | Great Britain..... | 204/49 |

## OTHER PUBLICATIONS

Endicott et al., Plating, Vol. 43, No. 1, p. 47 Jan. 1966

Primary Examiner—F. C. Edmundson  
Attorney—McGlew and Toren

[57]

## ABSTRACT

Known nickel plating baths can have large amounts of chloride incorporated in them. An improved nickel plating bath is described which has water-soluble bromide in it, preferably many times the weight of nickel present. The bath can include other electrodepositable metals besides nickel, so that the electrodeposition of hard nickel alloys can also be accomplished. The main result of the high bromide formulations proposed is to give deposits of nickel or its alloys which are notably free from stress. Many examples of nickel plating baths are given.

9 Claims, No Drawings

## ELECTRODEPOSITION OF NICKEL

This invention relates to the electrodeposition of nickel and nickel-containing alloys and is particularly concerned with providing an improved method of forming electrodeposits of nickel or of nickel alloys.

Nickel electroplating commonly uses, as the electrolytic bath, a solution of a nickel salt, e.g. nickel sulphate or sulphamate or nickel chloride, other components being included to produce a harder deposit or to reduce stress or to improve the performance of the electrolytic process. The production of a harder deposit normally involves the inclusion in the plating bath of a source of one or more metal ions in addition to nickel ions, so that more than one metal is plated out and the deposit is a nickel-based alloy. The reduction of stress and other improvements in the electrolytic process often involve the inclusion in the bath of components which do not plate out with the nickel, so that the deposit is nickel rather than a nickel alloy. Since essentially the same conditions apply to electroplating with nickel and to electroplating with nickel alloys, references to nickel plating herein are intended to refer generally to both nickel and nickel alloy deposits unless otherwise indicated.

It is known to include alkali metal chlorides in nickel plating baths. A considerable advance in nickel plating technique is described in British Patent specification No. 765,958, based upon the discovery that much larger amounts of sodium or potassium chloride than had previously been used gave improved throwing power and reduced stress. In an electrolytic bath according to British specification No. 765,958, the amount of sodium or potassium chloride is 7 to 12, and preferably 8, times the amount of nickel present in the nickel salt by weight.

It has now been discovered that an increase in throwing power and greater reduction in the tensile stress of the resultant nickel deposit can be obtained by incorporating in a nickel plating bath a large amount of a soluble bromide.

It has previously been proposed to incorporate bromides in nickel plating baths, for the purpose of promoting anode corrosion and so increasing anode efficiency. The bromide is usually introduced as nickel bromide, as in the Harstan nickel sulphamate process. The amount of bromide used up till now has been relatively small, e.g. up to one-third of the amount of nickel present by weight.

The present invention is based upon the use, in an acid nickel electrolyte including a source of nickel ions, an amount of bromide ions in excess of the amount stoichiometrically equivalent to the amount of nickel ions calculated as nickel bromide.

According to one aspect of this invention, a nickel plating bath comprises an aqueous solution containing at least one water-soluble nickel salt as a source of nickel ions and at least one water-soluble bromide as a source of bromide ions, the amount of the bromide preferably being 5 to 20 times and most preferably 10 times the amount of nickel by weight. Stated otherwise, the amount of bromide ions present is greater than if the nickel ions are derived from nickel bromide as the sole source of nickel ions in the bath.

The invention also provides a method of forming a nickel or nickel alloy electrodeposit, which may be an electroform, which comprises electrolyzing a plating bath of the composition just defined.

The benefits of the present invention are obtained with any bromide which has the essential requirements of being water-soluble and of not containing any ions which might adversely affect the performance of the bath. For example, the invention can be carried out both with sodium bromide and with potassium bromide. Moreover, the other alkali metal bromides and ammonium bromide can be used. It is surprising that bromides are effective in the way now discovered, for it has been found that sodium and potassium iodides have no comparable effect to that of the corresponding bromides.

The electrodeposit or electroform formed with a plating bath according to this invention can either be nickel or a nickel-based alloy. The requisite source of nickel ions can, if

desired, be provided wholly or partly as nickel bromide, which also contributes to the source of bromide ions also needed, though in this case additional bromide ions must be provided. Any other water-soluble nickel compound can also provide the source of nickel ions, though for most practical baths it is constituted by nickel chloride.

The source of bromide ions is preferably provided by sodium bromide, which is the water-soluble bromide most readily available. The other alkali metal bromides, which are regarded as comprising those of potassium, ammonium, lithium, rubidium and caesium for the purposes of this invention are also eminently suitable, though the latter three are somewhat costly. More than one bromide can be provided in the same bath if desired.

The acidity of the plating bath is important and in practice the pH of the bath should not normally be above 5.0 and, for most purposes, not above 4.0. A preferred range of pH is 1.8-4.0, the most suitable pH usually being about 3.5; higher pH's up to 4.5 are suitable if the bath is formulated so as to produce an alloy deposit.

Other components of the bath besides the nickel and bromide ions can be incorporated in order to achieve a variety of different effects. Other electrodeposable metal ions which can be included are, for example, one or more of cobalt, iron, zinc, manganese, uranium, molybdenum and vanadium. The invention can be used for the electrodeposition of low-stress or even substantially stress-free nickel/cobalt, nickel/iron and other alloys.

Another advantageous feature of the invention consists in the optional inclusion in a nickel or nickel alloy bath of the invention of a small amount of sulphite ion, e.g. provided in the form of sodium sulphite. A suitable quantity is constituted by up to 0.6 g/l of sodium sulphite; larger concentrations are possible, but it is usually unnecessary to use them. The main benefit afforded is stress reduction in the resultant deposits; low stress, coupled with high throwing power and heat-resistance, are characteristic benefits of the invention; with the inclusion of sodium sulphite, the stress can be further reduced and it is possible to obtain deposits with virtually no stress or even with compressive stress.

Organic stress reducers, i.e. compounds which are known to have a reducing effect upon the stress in a deposit, may be incorporated in baths of the invention in order to augment the tendency of the bath to produce low-stress deposits or to ensure that stress is maintained sufficiently low. Suitable additives for this include saccharin, sodium naphthalene trisulphonate, sodium meta-benzene disulphonate and other conventional stress reducers.

The acid electrolyte of the invention serves to produce an evenly distributed nickel or alloy deposit over a wide current density range, without excessive over-growths; stated otherwise, the electrolyte has high throwing power.

Throwing power may be defined as the characteristic of a solution which determines the evenness with which a metal may be deposited from it. There are several methods of determining the throwing power of a solution, such as those based upon the Haring cell or the Field apparatus. The test used to determine the throwing power of the present invention is that which was used for the solution described in specification No. 765,958, namely: weighing the deposit per unit area at the extreme inside center of a 90° angular test piece consisting of two square faces 2 x 2 inches at right angles to each other, stopped off at the back, dividing this weight by the weight per unit area deposited on the extreme outside corners and multiplying the result by 100.

The deposits obtained by electrolyzing a bath according to the invention without conventional stress reducers are heat-resistant, for instance they are capable of being brazed. Heat-resistant deposits have hitherto only been obtained from solutions which have a low inherent stress, such as nickel sulphamate baths. Such solutions usually have a low throwing power and consequently produce deposits which have very uneven distribution with nodular over-growths. The invention for the

first time provides a bath capable of forming a nickel or nickel alloy deposit at high throwing power, the deposit being both heat-resistant and free from excessive stress.

A nickel deposit produced with a bath according to this invention typically has a Rockwell C hardness in the range of 20-30 Rc. Harder deposits can be obtained by modifying the bath composition and the conditions of operating and hardnesses of 50 Rc or even higher can be achieved. One effect of the inclusion of other electrodepositable ions besides nickel ions in the bath is to produce a nickel alloy deposit which is often characterized by greater hardness. Of the alloying constituents mentioned above, cobalt, manganese, molybdenum and vanadium and mixtures thereof, in particular, when incorporated in the high bromide bath of the invention, preferably as the respective chlorides, give hard alloy deposits. For example, 5 g/l of cobalt gives hardnesses up to 480 DPN and 0.1-0.5 g/l of manganese gives hardnesses up to 350 DPN.

The deposits have a very low stress, which can often be obtained without the use of organic stress reducers, and can be produced at relatively high current densities, e.g. up to 100 A.S.F. The plating bath of the invention can be used without agitation or with agitation, such as air agitation, stirring or rod movement.

Unlike known nickel plating solutions, the solutions of this invention provide a combination of good hardness, ductility and low stress characteristic of nickel deposited without the use of organic stress reducers.

Further, it has been found that in the event of a failure of the source of current during electroplating, it is possible to continue plating without the occurrence of laminations simply by reversing the polarity for a short period and then recommencing plating.

Typical plating bath compositions of the invention are as follows:

|                                  | g/l        |         |    |
|----------------------------------|------------|---------|----|
| Ni <sup>++</sup>                 | 10-60      |         |    |
| H <sub>3</sub> BO <sub>3</sub>   | 32         | (25-40) | 40 |
| Br e.g. provided as NaBr or KBr) | 100-600    |         |    |
| pH                               | 3.0-4.0    |         |    |
| Operating temperature            | 18°-50° C. |         |    |

Unlike the high chloride bath described in specification No. 765,958, the high bromide bath of this invention can be used to plate directly on to most substrates, including aluminum, and a throwing power figure of about 50 or more is given.

In order that the invention may be readily understood, the following examples give details of the composition of a variety of plating baths according to the invention, together with details of the operating conditions employed in carrying out the method of electrodeposition of the invention using such baths and with details of the properties of the deposits obtained.

#### EXAMPLE 1

A bath was made up as an aqueous solution of the following 60 composition:

|                         | g/l |  |
|-------------------------|-----|--|
| Ni                      | 30  |  |
| Sodium bromide          | 300 |  |
| Boric acid              | 32  |  |
| Co (as cobalt chloride) | 5   |  |

The bath had a pH of 3.5 and was operated at 40° C. at a current density of up to 40 A.S.F. in still conditions and up to 80 A.S.F. with air or other agitation.

A fine-grained, hard, ductile and low-stress deposit of nickel alloyed with cobalt was obtained.

The following examples 2-11 were carried out similarly to Example 1, using an operating temperature of 40° C. and a current density ranging from 20-300 A.S.F., the pH and other operating conditions and the nature of the deposit being set out in the table.

#### EXAMPLE 2

|    | g/l              |     |
|----|------------------|-----|
| 10 | Nickel chloride  | 122 |
|    | Boric acid       | 32  |
|    | Ammonium bromide | 200 |

#### EXAMPLE 3

|    | g/l             |     |
|----|-----------------|-----|
| 15 | Nickel sulphate | 144 |
|    | Boric acid      | 32  |
|    | Sodium bromide  | 200 |
|    | Sodium sulphite | 0.5 |

#### EXAMPLE 4

|    | g/l             |      |
|----|-----------------|------|
| 25 | Nickel chloride | 122  |
|    | Boric acid      | 32   |
|    | Sodium bromide  | 200  |
|    | Uranyl acetate  | 0.04 |

#### EXAMPLE 5

|    | g/l              |      |
|----|------------------|------|
| 35 | Nickel sulphate  | 144  |
|    | Boric acid       | 32   |
|    | Sodium bromide   | 200  |
|    | Ferrous chloride | 10.7 |

#### EXAMPLE 6

|    | g/l             |      |
|----|-----------------|------|
| 45 | Nickel chloride | 122  |
|    | Boric acid      | 32   |
|    | Sodium bromide  | 200  |
|    | Zinc sulphate   | 0.44 |

#### EXAMPLE 7

|    | g/l             |      |
|----|-----------------|------|
| 50 | Nickel chloride | 122  |
|    | Boric acid      | 32   |
|    | Sodium bromide  | 200  |
|    | Zinc sulphate   | 0.44 |
|    | Sodium sulphite | 0.5  |

#### EXAMPLE 8

|    | g/l             |     |
|----|-----------------|-----|
| 65 | Nickel sulphate | 144 |
|    | Boric acid      | 32  |
|    | Sodium bromide  | 200 |
|    | Cobalt sulphate | 42  |
|    | Sodium sulphite | 0.5 |

#### EXAMPLE 9

|    | g/l              |     |
|----|------------------|-----|
| 70 | Nickel chloride  | 122 |
|    | Boric acid       | 32  |
|    | Sodium bromide   | 200 |
|    | Nickel phosphite | 0.5 |

#### EXAMPLE 10

|  | g/l |  |
|--|-----|--|
|--|-----|--|

|                |     |
|----------------|-----|
| Nickel bromide | 145 |
| Boric acid     | 32  |
| Sodium bromide | 400 |

## EXAMPLE 11

g/l

|                 |     |
|-----------------|-----|
| Nickel sulphate | 179 |
| Boric acid      | 32  |
| Sodium bromide  | 400 |

TABLE

| pH       | Deposit stress         | Plating test    |           |         |
|----------|------------------------|-----------------|-----------|---------|
|          |                        | Hardness,<br>Rc | Ductility | Surface |
| Example: |                        |                 |           |         |
| 2        | 3.5 Present            | 53              | Brittle   | Matt.   |
| 3        | 3.5 Slight compressive | 25              | Ductile   | Do.     |
| 4        | 3.5 Present            | 49.5            | Ductile   | Do.     |
| 5        | 2.0 do                 | 49              | do        | Br ght. |
| 6        | 3.5 do                 | 30              | do        | Do.     |
| 7        | 3.5 Absent             | 58.5            | Brittle   | Matt.   |
| 8        | 3.5 do                 | 58              | do        | Do.     |
| 9        | 3.5 Slight             | 22              | do        | Bright. |
| 10       | 2.5 do                 | 35              | Ductile   | Matt.   |
| 11       | 4.0 do                 | 27              | do        | Do.     |

I claim:

1. A method of manufacturing a self-supporting electroformed article by the electrodeposition of a metal selected from the group consisting of nickel and nickel based alloys, comprising

1. providing an electroforming bath of acidic pH and devoid of ammonium ions, which comprises an aqueous solution containing a nickel ion source and at least one water-soluble bromide as a source of bromide ions in which the weight of bromide in the aqueous solution is 5 to 20 times the weight of nickel,
2. immersing a substrate in the electroforming bath for receiving the desired electroforming deposit, and
3. electrolyzing said bath at a current density of up to 100 A.S.F. and at a bath temperature in the range of from 18° to 50° C. to thereby form on the substrate, at high throw-

5 ing power, an electroformed article free for excessive stress and being characterized by great hardness and good ductility.

2. A method as claimed in claim 1, wherein the pH value of the bath is between about 1.8 and 5.0.

3. A method as claimed in claim 1, wherein step (3) is continued until an electroformed article is obtained which has a minimum thickness of about 0.1 inch.

10 4. A method as claimed in claim 1, wherein the bath also contains at least one source of metal ions selected from the group of metals consisting of cobalt, iron, zinc, manganese, uranium, molybdenum and vanadium.

5. A method as claimed in claim 1, wherein the bath contains a source of sulphite ions.

6. A method as claimed in claim 5, wherein the source of sulphite ions is up to 0.6 g/l of sodium sulphite.

7. A method as claimed in claim 1, wherein step (3) is carried out in a static bath at a current density below about 50 A.S.F.

8. An electrolytic bath for the production of electroformed 35 nickel articles, comprising an acidic aqueous solution, devoid of ammonium ions, and comprising a source of nickel ions and at least one water-soluble bromide as a source of bromide ions, the weight of bromide being 5 to 20 times the weight of nickel.

9. An electrolytic bath as claimed in claim 8, wherein the pH value of the bath is between about 1.8 to 5.0.

\* \* \* \* \*

45

50

55

60

65

70

75